

Jan. 19, 1937.

G. W. BRYANT

2,068,032

PROCESS AND APPARATUS FOR THE MANUFACTURE OF RAYON

Filed March 27, 1935

4 Sheets-Sheet 1



INVENTOR  
George Willard Bryant  
BY  
Cooper, Kerr & Dunham  
ATTORNEYS

Jan. 19, 1937.

G. W. BRYANT

2,068,032

PROCESS AND APPARATUS FOR THE MANUFACTURE OF RAYON

Filed March 27, 1935

4 Sheets-Sheet 2



INVENTOR  
10 George Willard Bryant  
BY  
Cooper, Kerr & Dunham  
ATTORNEYS

Jan. 19, 1937.

G. W. BRYANT

2,068,032

PROCESS AND APPARATUS FOR THE MANUFACTURE OF RAYON

Filed March 27, 1935

4 Sheets-Sheet 3



Jan. 19, 1937.

G. W. BRYANT

2,068,032

PROCESS AND APPARATUS FOR THE MANUFACTURE OF RAYON

Filed March 27, 1935

4 Sheets-Sheet 4



INVENTOR  
*George Willard Bryant*  
BY  
Cooper, Kerr & Dunham  
ATTORNEYS

## UNITED STATES PATENT OFFICE

2,068,032

## PROCESS AND APPARATUS FOR THE MANUFACTURE OF RAYON

George Willard Bryant, Utica, N. Y., assignor to  
Skenandoa Rayon Corporation, Utica, N. Y., a  
corporation of Delaware

Application March 27, 1935, Serial No. 13,200

## 11 Claims. (Cl. 18—8)

This invention relates to the manufacture of rayon or artificial silk, and particularly to a new and improved process and apparatus for manufacturing rayon yarn.

5 My improved process includes a novel method of treating rayon in cake form, after the rayon yarn cakes have been washed or otherwise purified, to improve the dyeing and other qualities of the yarn, and particularly the dyeing properties 10 of rayon fabric made therefrom. My improved apparatus includes a novel machine for treatment of a rayon yarn cake after it has been washed or otherwise purified or liquid or fluid treated, but before it is dried.

15 An object of the invention is to provide a method and apparatus for manufacturing rayon yarn which, when fabricated, results in a rayon fabric having improved uniformity of dyeing properties.

20 Other objects of the invention are to provide a method and apparatus for manufacturing rayon yarn having improved uniformity of elasticity, crinkle, denier, strength and dyeing properties, the latter especially after fabrication of the 25 yarn; to provide a rayon yarn cake in which, when dried, the yarn throughout the cake has a substantially uniform "superficial elasticity" or "crinkle"; and to provide a substantially annular and undistorted rayon yarn cake in which the 30 yarn is free to contract in a substantially uniform manner and to a substantially uniform degree throughout all parts of the cake, during the drying operation.

35 Other objects of the invention will appear from the following description, and from the drawings and claims.

A result of my invention is to produce an improved rayon yarn, and a rayon yarn cake composed thereof, in which the yarn throughout the 40 cake has a substantially uniform "dye index", and possesses the important property of dyeing in a substantially uniform manner, not only before but, more particularly, after, fabrication of the yarn, and in which the rayon yarn has improved uniformity of elasticity, "crinkle", "wave", 45 and other desirable physical properties in addition to its improved uniformity of dyeing quality. To the ends stated a substantially uniform "superficial" elasticity or "crinkle" or "waviness", is 50 imparted to the yarn in all parts of the yarn cake and is thereafter preferably "set" or fixed in the yarn.

55 An advantage of the present invention is that, throughout the entire process, the yarn cake is

maintained in substantially annular and undistorted form.

Other results and desirable features of my invention will appear from the following description. 5

In the manufacture of rayon in this country a process commonly employed is the centrifugal one, sometimes referred to as "pot-spinning" or "bucket-spinning". As a result of this spinning process there is produced in the spinning pot or 10 "bucket", a "cake" of spun and twisted rayon yarn or fibre. In the case of the viscose process, with reference to which I shall more particularly describe my invention, this cake is composed partly of the twisted rayon fibres themselves, and 15 partly of various salts, acids and other impurities carried over by the fibres from the coagulating "spinning bath" through which the filaments are passed on their way to the spinning bucket, or resulting from decomposition of the viscose. 20 In order to complete the manufacture of the rayon it is necessary to subject the spun fibres to various purifying and drying treatments, sometimes referred to as "processing". In the viscose process, these treatments commonly include 25 "aging" the fibre, then washing to remove salts and other impurities, desulphuring, bleaching, further washing, soaping, hydroextracting, and finally drying the fibre or thread before it is wound into the form of a cone or other package 30 in which it is to be sold, or from which it is to be fabricated. Dyeing is ordinarily performed after 35 fabrication of the finished thread.

The present invention is applicable to, and may be used in connection with, the process and apparatus described in United States Patent No. 1,973,953, patented September 18, 1934 on application of Beirne Gordon, Jr.

The usual and conventional form and shape for a rayon yarn (sometimes called "fibre" or "thread") cake, when it is spun, which shape is ordinarily retained after the cake is "doffed" from the spinning pot (sometimes called the "box" or "bucket"), is that of the hollow frustum of a cone. So far as I know, such hollow frustro-conical yarn cakes (as illustrated, for example, in the drawings of the said Patent No. 1,973,953), are the type commonly spun in this country, although in certain foreign countries it has, from time to time, been proposed or attempted to spin a straight-walled or cylindrical (hollow) cake. 45 50 55

In accord with my present invention, and in order to overcome the foregoing and other difficulties, and to produce a rayon yarn susceptible 55

of being fabricated into a rayon fabric having high uniformity of dyeing quality, and having the other desirable properties and qualities previously described, I prefer to proceed according to 5 the following illustrative example:

I first spin a rayon yarn cake by suitable means (of which an example is described in the specification of the previously referred-to United States Patent No. 1,973,953), and then proceed to wash 10 and otherwise purify and treat or "process" the spun yarn cake in the manner described and claimed in that patent. I have found that during this and the treatment subsequently to be described, it is desirable and helpful to have the 15 yarn cake enclosed in an elastic fabric stocking or sleeve, in the manner described and claimed in United States Patent No. 2,002,481 to Beirne Gordon, Jr., and Harold J. V. Michel, patented May 21, 1935. After the yarn cake has been subjected to the desired purification and "process- 20 ing" treatments, it is inserted in the larger end of a reducing member having the form of a reducing die or "reducing tube". This member (or its internal bore formed by the ribs, to be pres- 25 ently described), is tapered in such a manner as to reduce the diameter of a yarn cake forced therethrough, as hereafter described. The tube is, preferably, open at both ends, and, in the pre- 30 ferred embodiment of my invention, is provided, on its interior surface, with a series of inwardly 35 projecting ribs or "flutings". These ribs are ar- ranged to radially indent or corrugate the yarn cake, and more particularly the outer surface thereof, in the desired manner hereafter described 40 in greater detail, without buckling the cake or 45 distorting it from its original substantially annular form. The yarn cake is then (as by means of a suitable plunger) forced through the tapered, fluted "reducing tube", with the result that the 50 cake is simultaneously reduced in diameter, and "crimped" or corrugated from its outer surface inwardly. The arrangement and proportions of the tube, its length, and the size, shape and taper of the internal ribs, are all coordinated in such a 55 manner (as hereafter particularly illustrated) that corrugations or flutings are introduced into the yarn cake from the outside inwardly. When the operation is completed, it is preferable that the corrugations are deepest in the outer layers 60 of the yarn, and decrease in size and depth as they approach the inner wall of the yarn cake. The reduced-diameter, corrugated yarn cake, after being forced along the "reducing tube", may 65 be discharged from the smaller end of the tube, and is still annular in form, but is provided with corrugations, particularly in its outer surface. It 70 is then transferred to and placed in a centrifugal bucket or "whizzer", of such diameter as just to receive the reduced-diameter cake. In making this transfer, use may be made of the collar here- 75 after described. In the whizzing apparatus the cake is subjected to the action of centrifugal force, during which operation it is not only maintained in substantially its original annular form, but even the yarn in the corrugations is thrown out- 80 wardly against the inner wall of the whizzing pot, by the centrifugal force. Some degree of hydro- extraction is also accomplished, whereby a part of the liquid is extracted from the cake by the 85 centrifugal force, and the subsequent drying operation is facilitated. The cake still retains, however, a considerable quantity of liquid, usually water, which must be removed by drying, com- 90 monly performed in a suitable oven. Before the cake is dried, the centrifugal action of the "whiz- 95

zer" (centrifugal bucket) has almost completely eliminated the corrugations produced in the outer wall of the cake by the ribs of the "reducing tube", changing the corrugations into sharp "crimps" or reverse bends. Throughout the process the 5 cake is maintained undistorted and substantially annular in form. But because the diameter has been substantially reduced throughout the cake, the yarn in all parts of the cake is free to contract in a substantially uniform manner, and this 10 is facilitated by the "crimps" remaining in the outer part of the cake after whizzing. A difficulty arising in previously suggested methods of yarn cake treatment and drying (namely that the yarn in the outer portion of the cake is subjected to 15 undue tension upon drying, while the yarn in the inner portions of the cake is free to contract without being subjected to undue tension, thus producing a yarn having non-uniform "crinkle", "wave", "superficial elasticity" and other proper- 20 ties), is thus overcome by my invention, accord- 25 ing to which the yarn cake is maintained in its annular shape and form before and during drying. Thus when shinkage subsequently occurs in the drying operation, there are no "hard spots" or 30 other non-uniform sections in the yarn, which is sometimes the case when the yarn is pulled tightly across the outwardly extending portions of a de- 35 formed, distorted or flattened yarn cake. There thus results, from the use of my invention, a 40 rayon yarn having high uniformity of "superfi- 45 cial elasticity", "wave" and "crinkle", as well as other desirable physical properties, and which, upon fabrication, produces a rayon fabric which may be dyed with improved uniformity and even- 50 ness, is substantially free from variations in color or shade, and is not subject to dyeing streaks or abrupt changes in appearance.

I shall now describe, by way of illustration, what 45 is at present the preferred form of my invention and method of practicing the same (being the best form of the method and apparatus now known to me), in greater detail in connection with the accompanying drawings, in which:

Fig. 1 is a side elevation, partly in section, of 45 the apparatus;

Fig. 2 is an end view, in elevation, of the ap- 50 paratus;

Fig. 3 is a detailed sectional view of the die- 55 like member or "reducing tube" with the plunger and a yarn cake therein;

Fig. 4 is a top plan view of the reducing die member shown in Fig. 3;

Fig. 5 is a sectional view taken on the line 55 5-5 of Fig. 3;

Figs. 6 and 7 are, respectively, a plan view and 60 an elevation, the latter partly in section, of a yarn cake after it is spun but before it is passed through the reducing die;

Fig. 8 is a plan view, diagrammatic in nature, 65 of the yarn cake after it has passed through and emerged from the reducing tube;

Fig. 9 is a diagrammatic plan view of the yarn 70 cake after it has been centrifugally treated;

Fig. 10 is an elevation, partly in section, of a 75 suitable form of centrifuging apparatus, for cen- trifugal treatment of the yarn cake after it has emerged from the reducing die;

Fig. 11 shows a modification of the apparatus, 80 partly in section, in which the plunger is oper- 70 ated by a compressed air ram; and

Fig. 12 is a detailed view, partly in section, of 85 the air ram mechanism.

Referring now more particularly to Figures 1 and 2, the cake reducing tube or die-like mem- 90

ber, 10, is shown arranged in vertical position, and provided with top and bottom openings, 10a and 10b. This die member is, of course, hollow or tubular in form, and is provided with ribs 11, 5 upon its inner face, and projecting radially inward from the face of the tube. The whole die member may conveniently be formed of a casting of brass, bronze or steel, polished on its inner face, and chromium plated to give a smooth finish and hard wearing surface.

The member 10 is supported on a frame or base 12, above which is arranged a suitable superstructure or framework 13. Affixed to the latter are an upper and a lower guide member, 14 and 15, respectively, in which is journaled the vertical rod 16, attached at its lower end to the plunger 17. The latter is arranged in the form of a spider, with radially extending fingers 18 (see Figures 3 and 4). The plunger and fingers are 20 so proportioned as to fit between the ribs 11 of the reducing tube, so that the plunger is free to pass to the bottom of the tube and eject the yarn cake therefrom.

For actuating the plunger 17 there is provided 25 a lever 19 hinged at 20 to the bracket 21 and provided with a slotted fork 22. The slots 22a in this fork receive and engage the pin 23 passing transversely through the vertical rod 16 upon which the plunger is carried. A handle 24 may 30 be provided at the outer end of the lever 19 and in addition, if desired, a counterweight, 25, suitably arranged upon a cord, 26, running over pulleys, 27.

In Figure 1 the reducing tube is shown in section with a yarn cake 28 forced part way through the tube.

Referring now more particularly to Figures 3, 4 and 5, the details of the die member 10 are shown, together with cross-sectional views (see 40 Figures 3 and 5) of a yarn cake 28 in progress therethrough. The initial position of the yarn cake is shown by the dotted lines 29, the dimensions of the reducing tube, at the inlet aperture 10a, being such that a spun yarn cake is received 45 and held therein in a position to permit entry of the plunger. The cake may be inserted in the reducing tube either small end first or large end first, depending, in part, upon the degree of axial compression desired. Discharge of the cake from 50 the lower end of the tube is facilitated by inserting the cake large end down.

Upon application of axial compression to the cake, by means of the plunger 17, the cake is forced downwardly and subjected to simultaneous 55 compression in the direction of its axis and radial indentation by the action of the ribs 11. If desired, the lower portion of the ribs 11 may be somewhat relieved for a few inches from the bottom, as at 11a, in order to permit somewhat freer passage and ejection of the yarn cake.

Figure 4 shows a plan view of the reducing die 10, with its co-operating plunger 17; and in Figure 5 there is shown, in horizontal cross-section, the die 10 and a yarn cake 28 in process of simultaneous radial indentation and axial compression, the cake being in the position shown by the full lines in Figure 3.

After the yarn cake has been ejected from the lower end of the reducing tube 10, it is transferred to the centrifuging pot or "whizzer" shown in Figure 10. This part of the apparatus may suitably include an electric motor 30 encased in a suitable protective hood 31, as illustrated. The motor is provided with a vertical shaft 32, having 75 at its upper end a vertical spindle 33, upon which

there is fitted an adaptor member 34, fitting into a suitable bushing 35. The latter is integral with the base 36 of the centrifugal "whizzing pot" or "whizzer" 37. The construction of the adaptor 34, and its cooperating bushing 35, may suitably be that described and claimed in United States Letters Patent No. 1,948,834 to Walter C. Volk, patented February 27, 1934. The whizzing pot 37 is provided with an apertured cover 38, held in place by an expanding bent wire spring member 39, arranged to snap into the groove 40 provided for the purpose, thus locking the cover into place during whizzing of the cake. Due to the fact that liquid is thrown off from the cake during the whizzing operation, 10 the whole apparatus is preferably encased in a box or other suitable enclosure 41, provided with a hinged lid 42, and a drain channel 43, through which liquid extracted from the cake may run off and be discharged.

The centrifuge pot 37 is circular in plan and in horizontal cross-section, and its interior diameter is preferably such that the yarn cake, after emerging from the reducing die, and upon being placed in the centrifuge pot, makes close contact with the latter, at the outer surface 44 of the cake. When it emerges from the die, the cake is substantially parallel-sided, and the centrifuge pot may, also, have parallel walls. However, a slight taper facilitates introduction and removal of the cake. The action of the centrifugal force is such that during the whizzing operation the yarn in the outer portions of the cake, even in the radial indentations 45 (see Figure 8), 20 is forced as much as possible into contact with the inner wall of the whizzing pot. Thus the yarn in the indentations 45 is thrown outwardly against the wall of the pot, but, since the periphery of the yarn cake 28, measured along its outer contour, and including the radial indentations 40 45, is substantially greater than the inner periphery of the pot 37 (the yarn cake having been substantially reduced in diameter by its passage through the die-member 10), the net result of the centrifuging operation is to produce 50 a yarn cake, still substantially annular in form but in which, due to the fact that the individual threads or yarn fibres are longer than the circumference of the cake in which they lie, the threads have, throughout the cake, a desired and desirable "crinkle" or "wavy structure", as heretofore described. This "crinkle" or "wave" permits the yarn to contract with substantial uniformity when dried, in cake form, after the centrifuging is completed and the excess "crinkle", not taken up by contraction, is set in the yarn, as hereafter described. The resulting yarn has been found to have improved uniformity of dyeing quality, particularly when fabric made therefrom is dyed subsequent to fabrication.

The form of the cake, in plan view, after completion of the centrifuging operation, is shown diagrammatically in Figure 9.

The operation of the apparatus is, briefly, as follows:

The rayon yarn cake 28, after having been spun in a centrifugal spinning bucket, is removed therefrom and enclosed in an elastic fabric protecting "stocking" 47 (see Figures 7 and 10). It is then suitably "processed" and purified, by 70 washing and otherwise, preferably as described in United States Letters Patent No. 1,973,953, previously referred to. After such "processing" or purification treatment, the cake is transferred to the reducing die, 10, where it is inserted in the 75

mouth thereof, 10a. By operation of the plunger 17, by the mechanism described, the cake is forced through the reducing die. Upon removal therefrom, at the outlet 10b, the reduced-diameter cake, now radially indented and axially compressed, is transferred to the centrifuging apparatus shown in Figure 10, where it is centrifugally treated. It is then removed and dried, preferably in an oven, after which the fabric covering 10 47 may be turned back from the cake and the yarn wound into a cone or other suitable package for sale or fabrication.

Figures 6, 7, 8 and 9 illustrate, in somewhat diagrammatic manner, the size and configuration of the yarn cake at different stages of the process. It will be observed that the yarn cake, throughout the operations, retains its generally annular form and configuration, but that it is substantially reduced in diameter by passage through 20 the die 10 and that, as a result of the process, the cake has had artificial crimps or corrugations introduced therein, more particularly in the outer portions thereof, and, in general, decreasing in amplitude from the outside toward the 25 inside of the cake. Since the crinkle or wave normally tending to occur during the drying of the cake is more pronounced at and near the inner surface thereof, and is much less or substantially non-existent at the outer surface of 30 the cake, it will be seen that the artificially-introduced crinkle, decreasing from the outside inwardly, tends to compensate the normally occurring crinkle, decreasing from the inside outwardly, with the result that, after drying, there 35 is a substantially uniform degree of crinkle and wave in the yarn in all parts of the cake.

It is to be noted that it is not necessary, in order to practice my invention with success, that the crinkled yarn from the inside and outside 40 of the cake should be identical in appearance, as regards the shape, depth, size and frequency of the crinkles; it is, in general, sufficient if the yarn from the inside, outside, and all intermediate portions, of the cake possesses substantially 45 or approximately the same amount or degree of crinkle, or has substantially the same proportion of its length occupied thereby.

In the case of a yarn cake spun in a spinning bucket of the customary approximately six-inch 50 diameter, the following approximate dimensions, given by way of illustration, have been found to be satisfactory in commercial use, within the limits of commercial tolerance:

For the top outside diameter of the cake before it is passed through the reducing die, six and one-eighth inches; for the bottom outside diameter of the cake before it is passed through the reducing die, five and thirteen-sixteenths 55 inches; for the height of the cake before it is passed through the reducing die, three and one-fourth inches. The thickness of the wall of the cake may be about three-quarters of an inch. For the outside diameter of the cake after passing through the reducing die, five and seven-sixteenths 60 inches; for the top inside diameter of the "whizzer pot" 37, five and one-half inches. The difference permits the use of the celluloid collar hereafter described. For the top outside diameter of the cake after centrifuging in the whizzing pot, five and seven-sixteenths 65 inches; for the height of the cake after passage through the reducing die three and one-eighth inches. A suitable overall height of the reducing die is 70 about twenty-six inches with a top inside diam-

eter, inside the ribs 11, of six and one-quarter inches, and a bottom inside diameter, inside the ribs 11, of three and fifteen-sixteenths inches. The latter may be relieved about one-eighth of an inch, for a distance of about three inches from the bottom, to facilitate passage of the 5 cake.

In drying a yarn cake of the approximate dimensions given, there ordinarily occurs a substantial shrinkage in the yarn, which may be of 10 the order of as much as six per cent of its length, under the conditions herein stated. An important feature of my invention is that it may be so carried out as to permit such shrinkage to occur, in the drying of the yarn (subsequent to 15 the centrifugal extraction of liquid therefrom), without subjecting the yarn to the tension and stretching which might take place if my invention were not employed. When my invention is not employed, and it is attempted to dry the 20 yarn in cake form, it may happen that the yarn at or near the outside of the cake is subjected to considerable tension because of the shrinkage which occurs in drying, and such tension produces, or tends to produce, an undesirable alteration in the structure and physical properties of the yarn, resulting in non-uniformity of dyeing quality. Many previous attempts to overcome this difficulty due to shrinkage have proven 25 unsuccessful, and have resulted in "hard spots" 30 or straight sections in the yarn, due to non-uniformity of shrinkage and tension during drying. My invention, however, overcomes this as well as the other difficulties previously mentioned. 35

For the reasons just stated, it is desirable that the reduction in diameter of the yarn cake, by passing it through the reducing die as heretofore described, should be at least sufficient to allow for the shrinkage of the yarn which occurs during the drying thereof. Such is, in fact, the 40 case, with the figures and dimensions given above; the yarn cake is sufficiently reduced in diameter by the reducing operation, and the centrifuge pot is sufficiently less in diameter than the spinning pot, so that the "crimps" or waves 45 produced in the yarn comprise (in the preferred embodiment of my invention) at least as great, and preferably somewhat greater, a percentage of the length of the yarn as the yarn thereafter contracts during drying; that is, in the example 50 given above, the "crinkles" and "waves" occupy at least, and preferably more than, about six per cent of the length of the yarn. Thus the "crimps" and "waves" comprise at least a sufficient amount of the yarn to allow for the 55 shrinkage which occurs upon drying, and there is preferably a substantial excess in the crinkles over and above what is taken up by shrinkage in drying, so that the finally purified and dried 60 yarn, after shrinking to its fullest extent, is substantially uniformly crinkled and waved, has a substantially uniform extensibility and elasticity, and has a substantially uniform percentage of its 65 length taken up by crinkles and waves, in all parts of the yarn cake. Thus yarn from all 70 parts of the completed yarn cake has substantial uniformity of the properties stated. Such is the preferred method of practicing my invention, and is the result of the figures and dimensions herein given by way of example.

A further advantage of my invention is that, in forcing the yarn cake through the reducing die member or tube, 10 (see Figure 3), the cake is subjected to simultaneous radial and axial com- 75

pression. The ribs 11 not only make radial indentations in the yarn cake, but the resistance is such that the plunger 17, in forcing the cake through the die, exerts a substantial axial compressional force on the top of the cake, and the height of the cake is consequently somewhat reduced. By reference to Figure 7 it will be seen that the cake is built up from a series of criss-crossed threads, due to the vertical reciprocating motion of the guide funnel during spinning. This gives to the cake a so-called "diamond" structure where the successive layers of thread cross at a slight angle, as illustrated in the upper right-hand part of Figure 7. Now, the vertical compression of the cake, and its consequent reduction in height, tends to flatten the "diamonds" with the result that each convolution of yarn lies in a more nearly horizontal plane. Hence each given length of yarn occupies a shorter path in the cake, and has, consequently, a little greater freedom to contract upon drying. Thus by vertical compression of the cake, simultaneously with its radial compression, the yarn is given increased freedom of shrinkage during drying, and less radial compression is necessary than if the vertical compression were not also effected.

In order to facilitate introduction of the reduced cake, 28, into the whizzing pot 37, and removal therefrom, I have found that it is often desirable to employ a celluloid collar 46, around the cake. Such a collar 46 is shown in Figure 10. It may be perforated to permit escape of liquid extracted from the cake during the centrifugal process. However, such perforations are not essential, since the liquid may escape at the top of the collar 46, and around the edges of the cover 38.

The celluloid collar 46 performs the dual function of acting like a "shoehorn" in facilitating insertion of the cake, Figure 8, into the whizzing pot 37, as shown in Figure 10, and also facilitating the removal of the cake after it has been subjected to the centrifugal force. When such a celluloid collar 46 is employed, the inner diameter of the centrifugal pot 37 should be sufficiently greater than the outer diameter of the reduced-diameter cake to allow for the insertion of the collar. This is indicated in the measurements given above.

In connection with the removal of the cake from the pot after it has been centrifuged, I have observed that, in the absence of a removable collar about the cake, such as 46, it may be difficult or impossible to remove the cake from the pot, indicating the substantial absence of internal strain in the yarn cake, after the centrifugal operation. Such absence of strain or tension in the cake, after the whizzing is completed (when the cake has previously been reduced in diameter in accord with my invention) is another advantage arising from the use of my invention, because I have observed that, in the ordinary centrifugal treatment of a yarn cake, when my invention is not employed, the cake tends to shrink away from the walls of the centrifugal pot as soon as the latter is stopped, indicating that the fibres are under tension during the centrifugal operation.

Throughout the process, from the time the yarn cake is first spun until the centrifuging is completed and the cake is dried, I have found that it is desirable to have the cake encased in an elastic fabric stocking or sleeve, as already described. Such a protective fabric covering is indicated, diagrammatically, at 47 in Figure 7, 75 where it is shown partially broken away to ex-

pose the yarn threads beneath. It is also shown, in section, in Figure 10, and is shown or indicated in the other figures.

Figures 11 and 12 show a modification of the apparatus in which the plunger is operated by an air ram under control of a suitable valve.

In Figure 11 there is shown a side elevation of the apparatus with the air ram operating mechanism, and

Figure 12 shows an end view, in elevation, of the apparatus, partly in section, showing the details of the air ram and its control valve and pipes.

Referring to Figure 12, the cake reducing tube or die-like member 10, is shown supported on the frame or base 12. Above the cake reducing tube 10, and attached thereto by suitable means, is a bracket 48 provided with an air passage 58.

Into the top of the bracket 48, there is screw-threaded a cylinder 49, and over the top of this cylinder 49, there is screw-threaded a cap 50, provided with an air passage 59. At the top and bottom of the cylinder, 49, there are provided suitable gaskets 54. A piston 51 is disposed in this cylinder 49 and is attached to the top of a vertical rod 52, and held there securely by means of a nut 53. To the lower end of the vertical rod 52, there is attached the plunger 17, arranged in the form of a spider as described hereinabove.

On the under side of the bracket 48, a packing gland 55, with a suitable packing 55a, is arranged for the vertically reciprocating rod 52. On the inward sides of the bracket 48, there are provided a pair of bosses 56, having slots or grooves, 57, to act as a guide for the plunger 17; these slots or grooves are preferably extensions of certain of the grooves provided by the ribbed interior of the tube 10.

A pipe line 60 connects with the air passages 58 and 59, and is provided with needle valves 61; 40 preferably two of such needle valves are included, one for each of the air passages as shown. Intermediate the needle valves, the pipe line 60 contains a four way valve 62, which has a port 62a connected to the branch of the pipe line 60 leading to the air passage 58, another port 62b connected to the branch of the pipe line 60 leading to the air passage 59, another port connected with a compressed air supply pipe line 63, and an exhaust port 65. This four way valve is of 45 the usual construction, operated by a lever 64, and arranged so that in its first position port 62b is connected with the supply line 63 and port 62a with the exhaust port 65, and in its second position port 62b is connected with the exhaust port 65 and port 62a with the supply line 63. 50 55

The operation of this apparatus is as follows: The plunger 17 (and the connecting rod 52) is in its upper position, as shown; a yarn cake is inserted through either of the open sides of the bracket 48, below the plunger, and is dropped into the reducing tube 10, as described hereinabove. With the needle valves suitably opened and the four way valve 62 in its first position, compressed air is transmitted from the supply line 63, through the four way valve, port 62b, the upper branch of line 60 and its needle valve 61, and the passage 59, into the top of the cylinder 49, and forces down the piston 51, its connecting rod 52 and the plunger 17. This downward movement of the plunger forces the yarn cake through the tube 10, in the manner previously described in reference to Figures 1 to 8. During its downward stroke, the plunger is guided by the slots or grooves 57, and the dead air in the cylinder 49 below the piston 51 is 70 75

forced out by the latter and exhausted through the air passage 58, the lower branch of line 60 and its needle valve 61, port 62a, the four way valve, and the exhaust port 65 to the atmosphere.

5 As will now be understood, the lever 64 can then be shifted or reversed to its second position, whereupon compressed air is admitted through port 62a and the passage 58 into the lower end of the cylinder 49, and the piston 51 is thereby 10 forced up to its original position, together with its connecting rod 52 and the plunger 17. On this upward stroke the dead air above the piston is at the same time forced out and exhausted through the passage 59, port 62b and the exhaust port 65.

15 The apparatus is then ready for insertion of another yarn cake and for operation thereon, carried out in the same manner, and initiated by shifting or returning the lever 64 to its first 20 position, as explained hereinabove. As will also be understood, the speed of operation of the plunger can be controlled by the needle valves 61, which are adjusted to regulate the amount of air admitted to and exhausted from the cylinder 49.

25 The process and apparatus herein specifically illustrated and described are the best embodiments of my invention now known to me, but it is to be understood that the invention is not necessarily or specifically limited thereto, but may be carried out in other ways without departing from its spirit, and within the scope of the following claims.

I claim:

30 1. Apparatus for use in the manufacture of rayon, comprising, in combination, a die-like receptacle having upon its interior surface a plurality of inwardly projecting tapered ribs, the mouth of said receptacle being of such size and 35 shape as to receive and accommodate a rayon yarn cake, and the taper, configuration and arrangement of said ribs being such as to compress said cake radially, upon forcing the cake into the receptacle; and means for forcing a rayon 40 yarn cake along said receptacle to subject the cake to radial compression.

45 2. Apparatus for use in the manufacture of rayon yarn, comprising, in combination, a tubular receptacle, substantially circular in cross section; a plurality of spaced and tapered ribs projecting radially inward from the interior face of said receptacle; a mouth for said receptacle, of size and shape adapted to receive a rayon 50 yarn cake; the form, size, shape, configuration 55 and taper of said ribs being coordinated so as to radially to compress a yarn cake forced along said receptacle; a plunger cooperating with said tubular receptacle and adapted to force a yarn cake into and along the same; and cooperating 60 means for actuating said plunger.

65 3. Apparatus for use in the manufacture of rayon, comprising, in combination, a die-like tubular receptacle, substantially circular in cross section; a plurality of spaced, tapered ribs projecting radially inward from the interior wall of said receptacle; an opening in the larger end of said receptacle of such size and shape as to receive a rayon yarn cake; the form, size, shape, configuration and taper of said ribs being such 70 as radially to compress a rayon yarn cake, and simultaneously to introduce corrugations therein, when the yarn cake is forced along said receptacle; a plunger-like member cooperating with said die-like receptacle and adapted to force 75 a yarn cake through the same; and cooperating

means for actuating said plunger member, said means comprising a cylinder, a piston arranged for movement therein, means connecting said piston with said plunger member for advance and retraction of the plunger in accord with the motion of the piston, means for admitting fluid, under pressure, upon one side of said piston to advance the plunger and force the yarn cake along said receptacle, and means for admitting fluid, under pressure, upon the opposite side of 10 said piston to retract the plunger.

5 4. In an apparatus for use in the manufacture of rayon, the combination of a die-like member having a converging internal bore of cross-sectional configuration such that it is adapted to 15 engage the outer surface of a rayon yarn cake and reduce the diameter of the cake as it is forced along said die member, and cooperating means for forcing a rayon yarn cake along said 20 converging bore.

5 5. In a machine for use in the manufacture of rayon, in combination, a die-like member having converging internal ribs and a plunger for forcing a yarn cake along said die-like member.

25 6. In a process of manufacturing rayon yarn, the combination of steps which comprises first spinning a rayon yarn cake by the centrifugal spinning method, then treating the cake to purify the yarn while substantially maintaining the original form of the cake, indenting the cake 30 at its outer periphery while subjecting it to simultaneous radial and axial compression, and then drying the cake.

35 7. In a process of manufacturing rayon yarn, the combination of steps which comprises first spinning a rayon yarn cake by the centrifugal spinning method, then treating the cake to purify the yarn while substantially maintaining the original form of the cake, substantially reducing the diameter of the cake by subjecting it to simultaneous radial and axial compression, 40 centrifuging the reduced-diameter cake, and then drying the yarn.

45 8. A process of manufacturing rayon comprising first spinning an annular rayon yarn cake by the centrifugal spinning system; then treating the spun cake to free the yarn from impurities, while maintaining the annular form of the 50 yarn cake; then radially indenting the cake at a plurality of spaced points about its periphery while still maintaining the annular form of the cake but subjecting it to simultaneous radial and axial compression; centrifuging the cake to convert the radial indentations into crinkles in the 55 yarn; and drying the yarn in cake form.

60 9. In the manufacture of rayon by the centrifugal spinning method, the process of manufacturing rayon yarn adapted for fabrication, before being dyed, into rayon fabric susceptible of being dyed with high uniformity, which comprises, in combination, the steps of first spinning a hollow frusto-conical rayon yarn cake, substantially annular in cross-section, by the centrifugal spinning method; then treating the cake to free the 65 yarn from impurities, while maintaining the annular form of the cake; substantially reducing the diameter of the cake while subjecting it to compression in the direction of its axis and simultaneously introducing radial indentations therein, without substantially altering the annular form of the cake; forcing excess liquid 70 out of the cake; and further drying the yarn.

75 10. The process of manufacturing rayon yarn adapted for fabrication, before being dyed, into

rayon fabric having substantial uniformity of dyeing properties even when the dyed fabric includes yarn from a plurality of yarn cakes, which comprises the steps of first spinning a substantially annular rayon yarn cake by the centrifugal spinning system; then treating the spun cake to free the yarn from impurities, while maintaining the substantially annular form of the cake; and then, without buckling the cake or materially distorting or deforming it from its original substantially annular form, substantially reducing the diameter thereof while simultaneously applying axial compression thereto; centrifuging the reduced-diameter cake; and then 10 drying the same, all while maintaining the original substantially annular form of the cake, and without any material deformation thereof.

11. The process of manufacturing rayon which comprises first spinning a substantially annular rayon yarn cake by the centrifugal spinning system; then treating the spun cake to free the yarn from impurities, while maintaining the substantially annular form of the cake; reducing the diameter of the cake by an amount sufficient to permit subsequent drying of the yarn in the cake without subjecting the yarn to substantial tension due to shrinkage occurring during drying, while simultaneously applying axial compression to the yarn cake; and drying the yarn while still contained in the reduced-diameter cake. 15

GEORGE WILLARD BRYANT. 15